

## UNITED STATES PATENT OFFICE.

ALBERT IVAN GATES WARREN, OF CATERHAM VALLEY, SURREY, ENGLAND, AS  
SIGNOR TO CATERHAM WORKS LIMITED, OF LONDON, ENGLAND, A COMPANY REG-  
ISTERED UNDER BRITISH LAW.

METHOD OF AND MEANS FOR PRODUCING METALLIZED SURFACES ON RUBBER  
COMPOUNDS CONTAINING SULPHUR.

No Drawing. Application filed December 5, 1922. Serial No. 605,072.

To all whom it may concern:

Be it known that I, ALBERT IVAN GATES WARREN, a subject of the King of Great Britain and Ireland, residing at Winchester 5 House, 375 Croydon Road, Caterham Valley, county of Surrey, England, have invented a new and useful Method of and Means for Producing Metallized Surfaces on Rubber Compounds Containing Sulphur, of which

10 the following is a specification.

This invention relates to the production of metal surfaces on rubber compounds containing sulphur such as vulcanite or ebonite, or on substances consisting of admixtures 15 of materials but in which rubber containing sulphur predominates.

It is well known that such materials as ebonite and vulcanite in their raw or finished state have but small affinity for chemical 20 change under ordinary conditions of temperature and use and for this purpose are often deliberately chosen for many industrial applications.

In the present invention advantage is 25 taken of the fact that the sulphur present in the rubber compound is capable under given conditions of heat and time of combining with metals or metallic salts when in intimate contact therewith, the metal 30 or positive radicle of the salt being absorbed as a sulphide or analogous compound of sulphur, this combination being determined in its area by direct contact with the metal or metallic salt, and in its depth depending 35 upon the length of time during which contact is preserved over the critical temperature, and in the case of metallic salts the duration of hot immersion, the thickness 40 of deposit, and subsequent heat soaking process.

This metallic absorption is evidenced by 45 the formation of metallic sulphides which become apparent in and upon the external or skin surface of the article treated. According to this invention the article is then 50 subjected to a suitable decomposing agent to eliminate the sulphur radicle and leave a conducting surface upon which if desired electrodeposition of other metals can be 55 made thereafter in any known manner.

The metals preferably employed for this

contacting process are gold and silver or a mixture thereof or their salts or oxides, but most of the metals capable of forming sulphides or compounds with sulphur such as zinc, nickel and tin may be employed though the results of their use are neither so certain, reliable or desirable as is the case with gold or silver.

In operation and in the preferred form of carrying this invention into effect, the article to be manufactured (other than plates, sheets or the like flat surface articles) is determined in shape by a mould or matrix. Into this mould a metallic foil consisting of a mixture of gold and silver is inserted, the gold constituent being preferably from 10-25 per cent and the silver constituent preferably 90-75 per cent, depending upon the final surface of the article required. The foil is of but small thickness varying from  $1/1000''$  to  $1/20''$  in thickness, depending upon the mass or pattern of rubber-sulphur material with which it will contact. In any case the foil is by tooling, pressing, moulding or like mechanical means forced into intimate contact with the mould, and caused closely to engage the surfaces presented. The unvulcanized or partly vulcanized rubber-sulphur material is now pressed into engagement with the foil, care being taken that no air bubbles or particles of foreign matter are interposed between the two engaging surfaces, the rubber-sulphur mass completely filling the foil-faced mould. Pressure may be employed to ensure contact, but a rolling or pugging action is most beneficial for the purpose, or the mould may be placed under vacuum to remove air bubbles between the rubber material and the foil. The articles in contact in the mould are now placed in an apparatus and heat treated to a vulcanizing temperature, namely between 300 to 330° F. for a period of at least 60 minutes. The temperature and period of heating depend in some small measure upon the quality of rubber used and the extent of prior partial vulcanizations and may vary within reasonable limits. It is preferable, therefore, first to ascertain by experiment the actual temperature and period of heating required for each distinct

kind of vulcanizable rubber. When the foil covered mass is extracted from the vulcanizer, it is found that the foil in contact may easily be removed from the vulcanized article, and that an appreciable loss in weight of foil has taken place, the loss being accounted for by its absorption within the mass, and is evidenced as a sulphide or like sulphur compound of the metal in recent contiguity. The remaining foil is now stripped. At this stage the metallized and vulcanized rubber-sulphur compound will have assumed its definite and ultimate shape and can be thereafter handled as an entity. The article thus formed is treated to reduce the metallic sulphide surface to metal by an appropriate reagent such as by immersion in an electrolytic ammoniacal or copper cyanide bath. If an electrolytic ammonium nitrate bath be employed in which the article treated constitutes the cathode, only 6 seconds are required for a 5 volt difference of potential. The bath must be made of a saturated solution of ammonium nitrate crystals at 65° F. When the article so treated is removed an obvious metallic surface is apparent. This surface is then burnished with a fine scratch brush and is then ready for use, or can be thickened with a depositable metal. If copper cyanide is employed an electrolytic bath is prepared, on a basis of 8 ozs. Copper cyanide crystals to one gallon of water at 65° F., and after immersion of the article as the cathode for ten minutes or less at a difference of potential of 2-3 volts it is found that the sulphides are reduced leaving a metallic surface with traces of copper. If an entirely coppered surface is required it may be obtained by longer immersion in the same, or for economy and a very smooth coating it may be inserted in an electrolytic copper sulphate bath composed of 1 lb. of copper sulphate to the gallon and  $\frac{1}{2}$  oz. of sulphuric acid at 65° F. and pressure of  $\frac{1}{2}$  volt.

This process of reducing or decomposing to a metallic state the surface metallic salt, is of prime importance as otherwise stripping of the electro-deposited layer will ensue sooner or later, or the metal layer subsequently deposited will blacken or ultimately show traces of sulphur activity.

When metallic salts in lieu of foil are employed, the article made of rubber compound may be first moulded and vulcanized or partly vulcanized. The moulded article after the first vulcanization has the appearance of vulcanite or ebonite depending upon the rubber compound employed that is to say it is a definite stable article in its moulded form. It is now, after being cooled, coated with a metallic salt or oxide preferably a salt or oxide of silver or gold or a mixture thereof. Again, preferably the oxide of

silver ( $\text{Ag}_2\text{O}$ ) is employed and this must be carefully prepared for purity and be of very fine division. It is prepared for use by forming same into a liquid or paste, with a volatile medium such as chloroform and/or rectified spirits of turpentine. This preparation may be applied by spraying or painting, or the article if wholly to be coated may be dipped into the preparation. After a sufficient coating has been applied to that portion of the article to be metallized, the volatile constituent is allowed to evaporate. This may be achieved by placing the moulded article so prepared in a drying chamber or oven for a sufficient period of time. Usually when the volatile medium is an admixture of turpentine and chloroform half an hour to two hours is necessary dependent upon the thickness of coating applied. The article may be now replaced in its mould and returned to the vulcanizer for further and complete vulcanization.

Not every composition of vulcanizable rubber is capable of second vulcanization, but such classes are well known in the art and are easily obtainable.

It is found that the further vulcanization has the result of transforming the metallic salt or oxide applied into a sulphide so that after the article is removed from its heat treatment the silver oxide and/or gold salt has become chemically combined with the surface depth of the rubber compound, as a sulphide or analogous sulphur salt. Further decomposition of the sulphide may now be effected as previously described by placing the article in an electrolytic bath of ammonium nitrate or copper cyanide solution and this process of further reduction and decomposition herein termed metallization may in fact be carried out simultaneously with the process of plating, in case of the copper cyanide bath.

Alternatively original moulds may be coated with metallic salts or oxides in paste form prior to the first moulding operation in which case the moulded article after vulcanization has all the characteristics of metal absorption, as though a metal foil has been employed, the production of a metallic surface for later electro-deposition being made in the manner set out above. In all cases, care must be taken that surface sulphides produced in the heat treatment are reduced or as a last precaution removed mechanically as with the scratch brush before plating takes place, or the later deposition will be unsatisfactory and produce uneven surfaces which are not desirable, the object being to produce a pure metallic surface on the article, which metallization decreases in purity with depth.

It is found that when the metallic salts or oxides are applied in paste form as above described, to either the mould or the article,

there is sufficient penetration or absorption of metal into the rubber compound to prevent any tendency of this chemically combined layer cracking off. The metallic salt 5 coating paste, however, must be homogeneous and of equal thickness over the portions required to be metallized. Whilst the reducing or decomposing agents employed under electrolytic agency are those which have been found best for the purpose, the 10 invention is not necessarily limited in this respect. Any reducing or decomposing agent similarly employed which will obtain the desired reduction or decomposition to 15 a metallic surface in the final stages of metallization may be regarded as the chemical equivalent of those stated above. If reduction or decomposition takes place in the plating bath it is necessary to move the 20 cathode clips during the process of plating along the article to be plated, so that the required action takes place with as near as possible equal intensity over the whole area.

In cases where certain rubber masses appear 25 to react slowly with the metallic mediums or salts employed the formation of surface sulphides may be accelerated by spraying or coating the surface of the article with carbon disulphide and then applying 30 the metal or metal salt.

In like manner to the use of foil, and metallic oxides or salts, finely comminuted metallic powders may be employed, the powder being applied either as a paste compounded with a volatile medium, or the article to be treated may be coated with a volatile medium and the metallic dust applied; or the metallic dust may alternatively be applied to the mould, the further process 40 of manufacture being otherwise identical with those described above.

This process of metallizing rubber compounds is particularly adapted inter alia to the production of gold covered dentures, 45 in the manufacture of which impressions of the mouth are taken in the usual way and moulds cast therefrom, in plaster of Paris. The mould is then preferably lined with foil and the dental rubber inserted until 50 the desired thickness of plate is built up, the teeth are inserted and the uppermost surface is then also covered with foil, and after vulcanization the denture is removed from the mould when cold and the foil 55 stripped therefrom. The denture is now immediately placed in the electrolytic ammonium nitrate bath as the cathode and treated for say 30 seconds to 1 minute at a pressure of 5 volts, the anode being 6" away 60 from the cathode. It is now removed, then washed, and scratch brushed being then ready for the final gold coating. This latter is applied in an ordinary electrolytic gold salt bath at a pressure of 1 volt until the 65 desired thickness of gold is deposited. It

is now burnished or polished and is ready for use, the final product has all the appearance and hygienic qualities of a gold plate without the disadvantage of cost, weight and liability to bend.

I claim:—

1. In a process for producing a metal surface on a rubber compound containing sulphur, the preliminary production of a metal sulphide on the surface by combination of a 70 metal with the sulphur in the rubber, and subsequently reducing such sulphide.

2. A process for producing a metal surface on a rubber compound containing sulphur, consisting of the application to the 75 surface of the rubber compound of a metal, heating the body to combine the metal and the sulphur, removal of uncombined metal, and reduction of the metal sulphide to metal, and electro-depositing further metal on the 80 metal derived from such reduction.

3. In a process for producing a metal surface on a rubber compound containing sulphur, the production of a metal sulphide by 85 heating the compound in contact with the metal, and subsequently reducing the sulphide to metal by electrolytic treatment.

4. A process for producing a metal surface on a body made of a rubber compound containing sulphur which consists in covering the body with gold and silver alloy, heating the body to vulcanize the same and to cause combination of some of the sulphur with the metal, removal of uncombined metal 90 reduction of the sulphide by treating the 100 body in an electrolytic bath and electro-depositing further metal on that derived from reduction.

5. In a process as claimed in claim 1, the particular method consisting of the use of a 105 silver oxide in a volatile medium to produce a surface layer, drying and subsequently heating to produce combination between the silver and the sulphur.

6. In a process as claimed in claim 1, the 110 particular method consisting in the use of finely comminuted metal powder to produce a surface layer, and subsequently heating to produce combination between the metal and the sulphur.

7. A process for producing a metal surface on a rubber compound containing sulphur, consisting of the application to the 115 surface of the rubber compound of a metal compound, heating the body to combine the metal and the sulphur, removal of uncombined metal, and reduction of the metal sulphide to metal, and electro-depositing further metal on the metal derived from such reduction.

8. In a process for producing a metal surface on a rubber compound containing sulphur, the production of a metal sulphide by 120 heating the compound in contact with the compound thereof, and subsequently reduc- 125

70

75

80

85

90

95

100

105

110

115

120

125

130

ing the sulphide to metal by electrolytic treatment.

9. A process for producing a metal surface on a rubber compound containing sulphur, consisting of the application to the surface of the rubber compound of a metal, heating the body to combine the metal and the sulphur, removal of uncombined metal,

and reduction of the metal sulphide to metal.

10. An article of manufacture comprising a rubber body having metal surfaces chemically combined therewith.

In witness whereof I affix my signature.

ALBERT IVAN GATES WARREN.